



US008393528B2

(12) **United States Patent**  
Richter et al.

(10) **Patent No.:** US 8,393,528 B2  
(45) **Date of Patent:** Mar. 12, 2013

(54) **METHOD FOR COATING A TURBINE BLADE**

(75) Inventors: **Karl-Hermann Richter**, Markt Indersdorf (DE); **Ulrich Knott**, Munich (DE); **Piotr Kowalczyk**, Munich (DE)

(73) Assignee: **MTU Aero Engines GmbH**, Munich (DE)

(\*) Notice: Subject to any disclaimer, the term of this patent is extended or adjusted under 35 U.S.C. 154(b) by 0 days.

(21) Appl. No.: **13/386,074**

(22) PCT Filed: **Jul. 8, 2010**

(86) PCT No.: **PCT/DE2010/000792**

§ 371 (c)(1),  
(2), (4) Date: **Feb. 6, 2012**

(87) PCT Pub. No.: **WO2011/009430**

PCT Pub. Date: **Jan. 27, 2011**

(65) **Prior Publication Data**

US 2012/0125980 A1 May 24, 2012

(30) **Foreign Application Priority Data**

Jul. 22, 2009 (DE) ..... 10 2009 034 168

(51) **Int. Cl.**  
**B23K 1/00** (2006.01)  
**B23K 1/19** (2006.01)

(52) **U.S. Cl.** ..... **228/262.9**; 228/262.31; 228/262.3; 228/262.71; 228/262.72

(58) **Field of Classification Search** ..... 228/262.3, 228/262.31, 262.71, 262.72, 262.9  
See application file for complete search history.

(56) **References Cited**

U.S. PATENT DOCUMENTS

|                 |   |         |                |       |          |
|-----------------|---|---------|----------------|-------|----------|
| 4,414,178 A     | * | 11/1983 | Smith et al.   | ..... | 420/444  |
| 5,198,308 A     |   | 3/1993  | Shetty         | ..... | 428/608  |
| 5,890,274 A     |   | 4/1999  | Clement et al. | ..... | 29/527.2 |
| 6,164,916 A     | * | 12/2000 | Frost et al.   | ..... | 416/189  |
| 6,638,639 B1    | * | 10/2003 | Burke et al.   | ..... | 428/583  |
| 2010/0297468 A1 |   | 11/2010 | Hecht et al.   | ..... | 428/615  |

FOREIGN PATENT DOCUMENTS

|    |                |        |
|----|----------------|--------|
| DE | 10 2007 048789 | 5/2009 |
| EP | 1 936 119      | 5/2000 |
| EP | 0 999 009      | 6/2008 |

\* cited by examiner

*Primary Examiner* — Erin Saad

(74) *Attorney, Agent, or Firm* — Davidson, Davidson & Kappel, LLC

(57) **ABSTRACT**

A method for hardfacing a metal component surface (14, 16), especially a shroud surface of a turbine blade made of a TiAl alloy, with at least one metal material (18, 20), in particular a Co—Cr alloy. The hardfacing coating is produced separately from the component surface and is then joined to the component surface in a high-temperature soldering process. A turbine blade including such a hardfacing coating, primarily in a shroud region (2).

**11 Claims, 1 Drawing Sheet**

**2**



2

Fig. 1



Fig. 2



Fig. 3



Fig. 4

## 1

## METHOD FOR COATING A TURBINE BLADE

The present invention relates to a method for providing a metallic component surface with a coating, and to a turbine blade provided with such a coating.

## BACKGROUND

The blades of low-pressure turbines are frequently made of nickel-based alloys or superalloys, such as, for example, IN 713, MAR 227 and B 1900. In order to reduce abrasion, the Z-shaped contact faces of their shrouds are usually hardfaced with cobalt-chromium alloys (Co—Cr alloys or Stellites®). The height of the hardfacing is typically 2 mm in the finished state. Methods typically used for producing the hardfacing are tungsten inert gas welding, micro-plasma welding and laser-beam welding. However, if the turbine blades are made of titanium aluminide material (TiAl), they cannot be provided with a Stellite® hardfacing, because this may cause the titanium aluminide to mix with the Stellite®, as a result of which brittle phases and cracks may form in the hardfacing and the titanium aluminide base material of the shroud.

## SUMMARY OF THE INVENTION

It is an object of the present invention to provide a method for providing a metallic component surface, in particular a contact face of a turbine blade made of a TiAl alloy, with a coating, which method overcomes the aforementioned disadvantages and makes it possible to achieve a hardfacing capable of withstanding stresses, and to provide a turbine blade provided with such a hardfacing.

In a method according to the present invention for providing a metallic component surface, in particular a shroud surface of a turbine blade made of a TiAl alloy, with a coating of a metallic material, in particular a Co—Cr alloy, initially, the component surface is manufactured undersized and a body is manufactured from the metallic material.

Then, the body is fixed to the component surface and joined thereto by high-temperature brazing.

The coating method of the present invention avoids material degradation and has the advantage that it allows the component surfaces to be provided with a stable coating or hardfacing without the risk of cracks forming in the hardfacing or in the base material of the component. Since the hardfacing is manufactured as a separate body, it is possible to achieve thicknesses which are cannot be achieved using alternative coating techniques, such as electroplating, PVD (Physical Vapor Deposition), or plasma spraying, so that the use of the method according to the present invention makes it possible to produce layer thicknesses greater than 2 mm.

In order to keep the effort for finishing the hardfacing low, it is advantageous for the body to already have at least two dimensions which correspond to two nominal dimensions of the hardfacing to be obtained before brazing is carried out. It is conceivable, for example, to manufacture the body such that it already has a nominal height and a nominal width of the hardfacing, so that finishing machining is performed only on lateral side surfaces defining the depth of the hardfacing.

In an exemplary embodiment, the body is indirectly joined to the component surface via an intermediate layer of a different material, in particular Inconel® 718 or nickel. The intermediate layer makes it possible to increase the bond of the body to the component because it allows the body and the component surface to be uniformly wetted by the braze material.

## 2

The intermediate layer may be in the form of a foil or plate and be applied first to the body. Then, the body is joined to the component surface via the intermediate layer.

Preferably, the intermediate layer is joined to the body at a 5 brazing temperature which is higher than a brazing temperature for joining the intermediate layer to the component surface. The brazing temperature for applying the intermediate layer to the body may, for example, be about 1050 °C. when a nickel-based braze material, such as a AMS 4777, is used, and the brazing temperature for joining the intermediate layer to the component surface may, for example, be equal to or less than 900 °C. when using a nickel-based braze material with a high content of noble metal, such as gold, silver or palladium (Au, Ag, Pd). A temperature in the range of about 900 °C. 10 is advantageous in particular when using titanium aluminide material, because this material is inherently unable to tolerate higher brazing temperatures.

In another exemplary embodiment, the body is initially 15 nickel-plated on its periphery and then joined to the component surface. Thus, the nickel layer acts, as it were, as an intermediate layer to improve bonding.

In a variant of the method without an intermediate layer, 20 brazing is accomplished by induction brazing, for example, in a high-vacuum furnace or in an inert gas atmosphere. Thus, 25 when titanium aluminide is used as the base material for the component, it is possible to set the brazing temperature to about 1050 °C. for a short period of time without the risk of damage to the base material. This makes it possible, for example, to use AMS 4777 braze material, which allows 30 uniform wetting of, for example, Stellite® bodies and TiAl components.

A turbine blade according to the present invention has a hardfacing applied thereto using the method of the present invention. The hardfacing is capable of withstanding stresses 35 and can have a height or thickness of several millimeters. Through application of the method according to the present invention, which preserves the integrity of the material, damage to the turbine material or to the hardfacing itself is prevented, as is any weakening of the turbine material or of the hardfacing caused by cracks forming upon application of the hardfacing.

Other advantageous exemplary embodiments of the present invention are the subject matter of further dependent claims.

## BRIEF DESCRIPTION OF THE DRAWINGS

Preferred exemplary embodiments of the present invention are described in greater detail with reference to schematic drawings, in which:

FIG. 1 is a top view of a shroud of a rotor blade of a fluid flow machine;

FIG. 2 is a cross-sectional view through a hardfaced region of a shroud provided with a first hardfacing according to the present invention;

FIG. 3 is a cross-sectional view through a hardfaced region of a shroud provided with a second hardfacing according to the present invention; and

FIG. 4 is a cross-sectional view through a hardfaced region 60 of a shroud provided with a third hardfacing according to the present invention.

## DETAILED DESCRIPTION

FIG. 1 shows a top view of a tip shroud 2 of a rotor blade of a fluid flow machine, in particular a gas turbine. Shroud 2 is made of a high-strength and high-temperature resistant tita-

num aluminide alloy (TiAl alloy). The shroud is substantially plate-like in shape and has two spaced-apart outer sealing lips or fins **6, 8** extending in the direction of rotation to minimize flow losses, and two Z-shaped side surfaces **10, 12**. Each of Z-shaped side surfaces **10, 12** defines a lateral gap to a shroud of an adjacent rotor blade and has a flat contact face **14, 16** to provide mutual support between it and an adjacent rotor blade for vibration damping purposes. In order to reduce mechanical wear, contact faces **14, 16** are each provided with a hardfacing **18, 20**.

Referring to FIG. 2, which shows a first exemplary embodiment of the invention, hardfacing **18, 20** has an approximately rectangular box-shaped body **22**. This body or chip **22** is preferably made of a Co—Cr alloy such as, for example, Stellite® 694, is of rectangular cross section and has a flat bottom surface **24** facing contact face **14** or **16** of shroud **2**.

In order to provide contact face **14** with hardfacing **18**, contact face **14** is manufactured such that it is suitably undersized. Body **22** is manufactured separately from shroud **2** using, for example, casting or sintering techniques. It has a height which corresponds to a nominal height of hardfacing **18**. The width of bottom surface **24** preferably corresponds to a width of contact face **14**.

Upon manufacture of body **22**, the body is fixed by its bottom surface **24** to contact face **14** and then brazed thereto, forming a large-area braze material layer **26**. Brazing is accomplished by induction brazing, for example, in a high-vacuum furnace or in an inert gas atmosphere at a temperature of about 1050 °C. using AMS 4777 nickel-based braze material, which is capable of uniformly wetting Stellite® contact face **24** and TiAl component surface **14**.

After body **22** is brazed to shroud **2**, hardfacing **18** is machined to its final dimensions. Since body **22** already has a width corresponding to contact face **14** and, in addition, the overall height of body **22** corresponds to the nominal height of hardfacing **18**, machining to final dimensions (e.g. by grinding) is only required to adjust the depth of body **22** to a depth of contact face **14**. Of course, body **22** may also be formed with oversized dimensions to compensate for component and assembly tolerances, in which case machining to final dimensions would also be necessary for the height and/or width of hardfacing **18**. It is also obvious that body **22** may be formed in such a way that it already has all the nominal dimensions of the hardfacing, thus eliminating the need for machining to final dimensions.

Referring to FIG. 3, which shows a second exemplary embodiment of hardfacing **18, 20**, body **22** may also be joined to contact face **14, 16** of shroud **2** via an intermediate layer **28**. Intermediate layer **28** is disposed between contact face **14** and bottom surface **24**, and serves to improve the bond of body **22** to shroud **2**. The intermediate layer is preferably made of a nickel-based alloy or superalloy, such as INCONEL® 718, and is formed as a thin plate or foil of constant thickness. Bottom surface **24** of body **22** and intermediate layer **28** each have a geometry that corresponds to contact face **14**, so that a maximum bonding area is created between contact face **14** and intermediate layer **28**, and between intermediate layer **28** and bottom surface **24**.

In order to provide contact face **14** with hardfacing **18**, contact face **14** is manufactured such that it is suitably undersized. Body **22** is manufactured separately from shroud **2**, and intermediate layer **28** is provided. The height of body **22** corresponds to the nominal height of hardfacing **18** minus the thickness of intermediate layer **28**. The width of bottom surface **24** preferably corresponds to the width of contact face **14**.

Preferably, intermediate layer **28** also has a width that corresponds to the width of the contact face.

Then, intermediate layer **28** is brazed to bottom surface **24**, forming a large-area braze material layer **30**. This is done at about 1050 °C. A preferred braze material is a nickel-based braze material, such as AMS 4777, because such material is capable of uniformly wetting both TiAl materials and Stellite® materials.

After intermediate layer **28** is applied to bottom surface **24**, body **22** is indirectly fixed to contact face **14** via intermediate layer **28**. Then, intermediate layer **28** is brazed to contact face **14**, forming a large-area braze material layer **32**. This is done at a temperature less than the temperature at which intermediate layer **28** is brazed to body **22**. Preferably, the temperature is selected to be less than or equal to 900 °C. A preferred braze material is nickel-based and has a high content of noble metal, such as gold, silver or palladium. Examples include Gapasil® 9, Palcusil® 10 and Palnisi® 10.

After body **22**; i.e., intermediate layer **28**, is brazed to shroud **2**, hardfacing **18** is machined to its final dimensions. Since body **22** and intermediate layer **28** already have a width corresponding to contact face **14** and, in addition, the overall height of body **22** including intermediate layer **28** corresponds to the nominal height of hardfacing **18**, machining of hardfacing **18** to final dimensions only needs to be done for one dimension, here the depth. Of course, body **22** and intermediate layer **28** may also be formed with oversized dimensions to compensate for component and assembly tolerances, in which case machining to final dimensions would also be necessary for the height and/or width of hardfacing **18**.

In accordance with the exemplary embodiment of hardfacing **18, 20** illustrated in FIG. 4, body **22** may also be coated with a nickel layer **34** on its periphery. In this case, the nickel layer on bottom surface **24** serves, as it were, as an intermediate layer to improve bonding. The geometry of body bottom surface **24** corresponds to the geometry of contact face **14** and **16**, respectively. The height of the body corresponds to the nominal height of hardfacing **18**.

In order to provide contact face **14** with hardfacing **18**, contact face **14** is manufactured such that it is suitably undersized. Body **22** is manufactured separately from shroud **2** and nickel-plated on its periphery. Because machining of hardfacing **18** to its nominal dimensions is no longer possible once the nickel layer is applied, body **22** already has the nominal dimensions of hardfacing **18** before its is nickel-plated. This means that prior to the application of the nickel layer, body **22** has a height corresponding to the nominal height of hardfacing **18**; and the width and depth of its bottom surface **24** correspond to the width and depth of contact face **14**. After body **22** is nickel-plated, it is fixed by its nickel-plated bottom surface **24** to contact face **14** and then brazed thereto by a braze material layer **36** at a temperature of about 900 °C.

Disclosed is a method for hardfacing a metallic component surface, in particular a shroud surface of a turbine blade made of a TiAl alloy, with at least one metallic material, in particular a Co—Cr alloy, in which method the hardfacing is produced separately from the component surface and subsequently joined thereto using a high-temperature brazing technique. Also disclosed is a turbine blade which is provided with such a hardfacing, especially in a shroud region.

What is claimed is:

1. A method for providing a TiAl-component surface with a coating of at least one metallic material comprising the steps of:  
manufacturing the component surface with undersized dimensions;

## 5

coating the component with the at least one metallic material, the step of coating including  
manufacturing a body composed of the at least one  
metallic material;  
fixing the body to the component surface; and  
joining the body to the component surface by brazing;  
wherein an intermediate layer of a different material is first  
applied to the body, and then the intermediate layer is  
joined to the component surface by the brazing, a brazing  
temperature for joining the intermediate layer to the  
component surface being less than or equal to 900° C.;  
and  
wherein the brazing includes joining the intermediate layer  
to the body at a first brazing temperature higher than the  
brazing temperature for joining the intermediate layer to  
the component surface.

2. The method as recited in claim 1 wherein prior to the  
joining, the body has at least two dimensions corresponding  
to two nominal dimensions of the coating.

3. The method as recited in claim 2 wherein subsequent to  
the brazing, the body is machined to final dimensions with  
respect to width and/or depth.

4. The method as recited in claim 1 wherein the brazing  
temperature for applying the intermediate layer to the body is  
about 1050° C.

5. The method as recited in claim 4 wherein the brazing  
includes using nickel-based braze materials with a high  
content of noble metal.

6. The method as recited in claim 5 wherein the noble  
metals include gold, silver or palladium.

## 6

7. The method as recited in claim 1 wherein the different  
material includes nickel, and wherein intermediate layer is  
applied to the body by nickel-plating the body on a periphery  
prior to joining the body to the component surface.

8. The method as recited in claim 1 wherein the at least one  
metallic material includes a Co—Cr alloy.

9. The method as recited in claim 8 wherein the different  
material includes Inconel® 718 or nickel.

10. The method as recited in claim 1 wherein the different  
material includes Inconel® 718 or nickel.

11. A method for providing a TiAl-shroud surface of a  
turbine blade with a coating of at least one metallic material  
comprising the steps of:

manufacturing the shroud surface with undersized dimen-  
sions;

coating the shroud surface with the at least one metallic  
material, the step of coating including  
manufacturing a body composed of the metallic mate-  
rial;

fixing the body to the shroud surface; and

joining the body to the shroud surface by brazing;  
wherein an intermediate layer of a different material is first  
applied to the body, and then the intermediate layer is  
joined to the shroud surface by the brazing, a brazing  
temperature for joining the intermediate layer to the  
shroud surface being less than or equal to 900° C.; and  
wherein the brazing includes joining the intermediate layer  
to the body at a first brazing temperature higher than the  
brazing temperature for joining the intermediate layer to  
the shroud surface.

\* \* \* \* \*